

Patented Oct. 4, 1932

1,880,411

# UNITED STATES PATENT OFFICE

ROBERT E. BURROUGHS, OF ROCHESTER, NEW YORK, ASSIGNOR TO EASTMAN KODAK COMPANY, OF ROCHESTER, NEW YORK, A CORPORATION OF NEW YORK

## ULTRA-VIOLET SENSITIVE PHOTOGRAPHIC ELEMENT

No Drawing.

Application filed May 6, 1931. Serial No. 535,576.

This invention relates to a photographic element which is sensitive to the extreme ultra-violet portion of the spectrum.

In modern industrial and scientific research spectro-photography plays a considerable part, and in this field the characteristics of various materials under the influence of ultra-violet radiations are of interest. Much of this kind of work is now done with the quartz spectrograph and measurements are made from the visible as far into the ultra-violet as is possible. This work is, of course, all done with the help of commercially obtainable photographic plates or films. The materials available have, however, introduced difficulties due largely to the fact that the gelatin in which the silver halide grains of the emulsion are embedded absorbs the radiations of very short wave lengths, thereby preventing their action upon the silver halide grains which in themselves are sensitive to the radiations.

A number of previous workers have attempted to overcome this drawback by incorporating in the emulsion a fluorescent substance. The purpose of such a substance in general is to transform the radiations of short waves into radiations of longer wave lengths which are not so strongly absorbed by the gelatin. In this way the invisible short wave lengths are changed into the longer visible wave lengths which are able to act upon the silver halide grains, as they are not absorbed by the gelatin. These radiations will usually be of a blue or greenish color.

I have found a material and a method which is particularly satisfactory for sensitizing a photographic plate or film to the extreme ultra-violet. The material which I use is ethyl-dihydro-collidine-dicarboxylate. This material is put on the surface of the emulsion in a very thin layer, and is removed by the subsequent treatment of the plate or film.

A satisfactory method of applying this thin coating is to bathe the plate for a few seconds in a solution of ethyl-dihydro-collidine-dicarboxylate. A suitable bath is the following:

Ethyl-dihydro-collidine-dicarboxylate 5 gm.  
Ethyl acetate 95 ."

The plate or film is dipped in this solution for a few seconds, withdrawn and slowly dried in a position such as to drain off as much of the solution as possible.

A plate or film treated as described is handled in the ordinary way. After drying it may be stored for some time before exposure. After exposure it is developed and fixed in the ordinary way. The crystals which remain on the emulsion after development are removed by washing the plate in alcohol or by brushing with a tuft of cotton during development.

The method of sensitizing to the ultra-violet as described has advantages over the older method of incorporating the fluorescent material in the emulsion, and by the present invention the sensitizer is completely removed without any additional steps and no trace of its presence is left in the emulsion after development and fixing. Plates or film sensitized in the manner described with ethyl-dihydro-collidine-dicarboxylate will show a sensitivity in the ultra-violet beyond 60 $\mu$ .

What I claim is:

1. A photo-sensitive gelatino silver halide layer comprising ethyl-dihydro-collidine-dicarboxylate.
2. A photographic element comprising a support, an emulsion layer containing silver halide, and on the surface of said emulsion layer a thin superficial coating of ethyl-dihydro-collidine-dicarboxylate.

Signed at Rochester, New York, this 28th day of April, 1931.

ROBERT E. BURROUGHS. 90